

# UNITED STATES PATENT OFFICE.

EMILE BRONNERT, OF NIEDERMORSCHWEILER, GERMANY, ASSIGNOR TO THE FIRM OF VEREINIGTE GLANZSTOFF-FABRIKEN A.-G., OF ELBERFELD, GERMANY.

## PROCESS FOR THE PRODUCTION OF SHAPED ARTICLES FROM COPPER-AMMONIUM CELLULOSE SOLUTION.

1,106,077.

Specification of Letters Patent. Patented Aug. 4, 1914.

No Drawing.

Application filed April 9, 1913. Serial No. 759,983.

*To all whom it may concern.:*

Be it known that I, EMILE BRONNERT, a subject of the Emperor of Germany, and a resident of Niedermorschweiler, near Mühlhausen, Germany, have invented certain new and useful Improvements in Processes for the Production of Shaped Articles from Copper-Ammonium Cellulose Solutions, of which the following is a specification.

10 The invention relates to a process and to a solution for precipitating cellulose from a cupra-ammonium solution, and aims to provide improvements therein.

It is well known from German Patent No. 186,387 that concentrated soda lye, especially when heated, acts as an excellent medium for precipitating cellulose from a cupra-ammonium solution thereof. Also that soda lye, for example, down to 5 per cent. NaOH content, acts as a precipitating medium, with the formation of copper sodium cellulose.

The rapidity of the precipitation is, naturally, proportionally less, the lower the alkali content of the precipitating bath. In the spinning of threads this is a disadvantage, since the drawing off of the thread takes place so much slower than otherwise. If it be attempted to employ a still weaker solution of alkali, then no proper precipitation occurs; accordingly when solutions of less than 5 per cent. alkali are used as a precipitating bath, the cupra-ammonium cellulose solution is expressed or squirted through wide openings from 0.50 to 1.00 millimeters into the alkaline solution in relatively thick streams, and suitable drawing-off devices employed to draw the precipitated cellulose into a very fine thread, 40 the drawn-out thread being then treated with stronger lye or acid for the purpose of thorough coagulation and hardening. This is the so-called "stretch-spinning" process. On the other hand, it is well known, for example, through the French Patent No. 379,000, that an addition of easily soluble salts permits of the use of weaker solutions of lye than when the soluble salts are not used.

50 By the present invention, it is shown that by the use of sodium lactate, or sodium glycolate, both of which are extremely easily soluble salts, the content of the precipitating bath in caustic alkali can be less-

ened to a very remarkable degree, without 55 reducing the precipitating power of the bath. There is directly attained, while using the above-described bath under increased temperature, and with only two and one-half per cent. caustic soda, threads so strong 60 that they can be wound up with the same speed as if they were threads from concentrated soda lye, a thing that is not possible with a solution containing so low a per cent. of soda lye alone.

65 The following example of the process is given: In concentrated solution of 100 cubic centimeters sodium lactate there is dissolved 2.5 grams of caustic soda. This is heated to 50° C. and employed as a precipitating 70 bath, into which a solution of cellulose in cupra-ammonium is squirted through suitable capillary tubes (of 0.16 millimeters to 0.22 millimeters for example), and the cellulose precipitated. The issuing threads may 75 be received upon winding spools or reels. On subsequent washing with water, for the purpose of removing the soda lye, it is found that the threads do not become Turkish blue, from the copper hydroxid separating out 80 upon the threads, as when lye alone is used or lye with common salt (sodium chlorid) but they become clear green-blue, as if concentrated soda lye and sugar had been employed, as in the process of German Patent 85 No. 208,472. This remarkable effect of the sodium lactate is explained by the fact that the lactic acid like the sugar and glycerin, in consequence of the hydroxyl-group contained therein, is capable of partly releasing 90 the copper from the thread and carrying it into the washing water; the lactic acid also in part receives the residue in the thread in fixed solution, which solution is clear. It is made clear from this state of affairs that 95 other salts also of hydroxy acids, such as glycol acid, tartaric acid, or citric acid, can be used with like success in the form of concentrated solution with the addition of a few percent of caustic soda.

100 With the aid of the process of the present invention there are attainable clear green articles, such as threads, filaments, or films poor in copper. After de-coppering, for example, with a usual acid, these products 105 are highly lustrous and of great strength and elasticity.

The utilization of the hydroxy-acid salts,

of course, does not exclude use at the same time of other materials, such, for example, as sugar and the like. The hydroxy-acid salts can, moreover, partially or wholly, be 5 incorporated in the cellulose solution.

The cellulose solution can also be so produced that copper-lactate or glycolate etc., is dissolved in ammonia, and then an equivalent amount of caustic alkali is added, and 10 then the cellulose is introduced.

What is claimed is:—

1. A process for the production of shaped articles from copper-ammonium cellulose solutions, comprising introducing a solution 15 of copper ammonium cellulose into a warm solution containing an alkali and a high concentration of a salt of an oxy-acid, thereby obtaining a precipitation of the cellulose.

2. A process for the production of shaped 20 articles from copper-ammonium cellulose solutions, comprising introducing a solution of copper ammonium cellulose into a warm solution containing a low concentration of an alkali and a high concentration of a salt

of an oxy-acid, thereby obtaining a precipitation of the cellulose. 25

3. A process for the production of shaped articles from copper-ammonium cellulose solutions, comprising introducing a solution of copper ammonium cellulose into a warm 30 solution containing approximately  $2\frac{1}{2}$  percent of an alkali and a high concentration of a salt of an oxy-acid, thereby obtaining a precipitation of the cellulose.

4. A process for the production of shaped 35 articles from copper-ammonium cellulose solutions, comprising introducing a solution of copper ammonium cellulose into a warm solution containing an alkali and a high concentration of a salt of lactic-acid, thereby 40 obtaining a precipitation of the cellulose.

In testimony that I claim the foregoing as my invention I have signed my name in presence of two subscribing witnesses.

EMILE BRONNERT.

Witnesses:

DAVID BRONNERT,  
ARNOLD ZUBER.